

## UNITED STATES PATENT OFFICE

2,640,812

## GREASE

William C. Bryant, Garfield, N. J., assignor to  
 Swan-Finch Oil Corporation, New York, N. Y.,  
 a corporation of New York

No Drawing. Application March 8, 1951,  
 Serial No. 214,651

12 Claims. (Cl. 252—33.6)

1

This invention relates to lubricants and more particularly to grease-like lubricants containing modified montmorillonite and another gelator serving to improve the results obtained by the use of montmorillonite alone.

The gelling of the organic fluids to form greases by modified montmorillonite, in which the sodium or part of the sodium has been replaced by a long chain secondary amine group is known. Such greases have been introduced on the market as Bentone greases. As stated in "The Institute Spokesman," May 1950, the official publication of the National Lubricating Grease Institute, page 13, Bentones are the reaction products of bentonite, or more accurately, montmorillonite, and various organic cations. Montmorillonite is a hydrous magnesium aluminum silicate with a micaceous structure and an exceptionally small ultimate particle size. It occurs customarily as the salt of the moderately strong acid. The montmorillonite used for the production of the Bentones is the Wyoming type in which the cation is predominantly sodium.

To prepare a Bentone, the montmorillonite is hydrated in a very dilute dispersion to separate the unit particles, and is purified by super-centrifugation to achieve complete removal of non-clay impurities. This step is resorted to since most montmorillonites in the crude state contain relatively large quantities of quartz which, if allowed to remain, would impart an abrasive character to the resulting product. The reactive sodium atoms of the unit plates are then replaced by organic cations and the product washed, filtered, dried, etc., to give the final Bentone. A suitable cation is ammonium.

By proper choice of the organic cation the properties of the resulting Bentone can be controlled. Use of a short chain alkyl ammonium salt gives a Bentone with slight organophilic properties and retention of a large part of the original hydrophilic properties. Increasing the chain length of the alkyl ammonium salt gives increasing organophilic properties. Use of a quaternary ammonium salt with two long chains, say, 16 to 18 carbon atoms each, gives a completely hydrophobic and organophilic Bentone, and greatly improves the heat stability.

The characteristic of lubricating greases made from the modified montmorillonite is the resistance of such greases to high temperatures. It is substantially impossible to melt such greases. In fact, such greases made from mineral oil and synthetic oil resist melting when heated beyond the ignition point of such oil.

Such greases are known to catalyze rusting of

ferrous metals. As stated in the above-mentioned article, such Bentone greases have weak characteristics and one of them is the lack of adequate rust-preventive properties; another one is the lack of resistance to oxidation. Another disadvantageous characteristic is the fact that the gel structure of such Bentone grease is so rigid as to preclude the release of oil from the mass regardless of temperature resulting in excessive wear of bearings because they are forced to run under starved lubrication conditions.

The usual rust inhibitors now generally recommended for use in industry are unsatisfactory for use with such Bentone greases. They have the property of diminishing the gel strength of the modified montmorillonite greases and do not satisfactorily prevent rusting; nor do they overcome the other faulty characteristics of the Bentone greases.

The principal object of the present invention, accordingly, is to provide an improved Bentone grease and grease base in which at least some of the above-mentioned difficulties are overcome.

In my copending application Serial No. 176,243, filed July 27, 1950, I have described and claimed a lubricating composition having in combination as ingredients a modified montmorillonite as a first gelator and a second gelator selected from a group of certain diamides and amic acids together with a lubricating vehicle. In the present application, I describe and claim a lubricating composition having a petroleum lubricant, a modified montmorillonite, and a long chain organic salt gelator, as more particularly described below.

The invention accordingly comprises the novel products, the specific embodiments of which are described hereinafter by way of example and in accordance with which I now prefer to practice the invention.

I have found in accordance with my invention that I may prepare a grease or lubricant base by providing a composition containing a substantial amount of a modified montmorillonite and a long chain organic salt gelator, dispersed in a petroleum lubricant. The organic salt gelator contains a straight chain of at least 8 carbon atoms and its salt-forming metal is lithium, sodium, calcium, barium or strontium. This organic salt may be a barium, strontium, sodium, calcium or lithium soap as found on the market or it may be a substance having the formula



where X is an alkali metal, R is selected from the group consisting of methylene groups having

a carbon chain length of 1 to 8 carbon atoms and the group



R<sub>1</sub> is an aliphatic radical of a carbon chain length of 4 to 18 carbon atoms, and R<sub>2</sub> is selected from the group consisting of hydrogen and an aliphatic radical of a carbon chain length of 4 to 18 carbon atoms; or it may be a substance having the formula

(B)



where M is an alkaline earth metal; R is selected from the group consisting of methylene groups having a carbon chain of 1 to 8 carbon atoms and the group



R<sub>2</sub> is an aliphatic radical of a carbon chain length of 4 to 18 carbon atoms, and R<sub>3</sub> is selected from the group consisting of hydrogen and an amic acid radical having the formula



These substances and the processes for making them are described and claimed in the copending application of William C. Bryant (the present applicant) and Anthony Giordano, Serial No. 80,328, filed March 8, 1949 now Patent No. 2,604,449. The substances falling under Formula (A) and Formula (B) above are derivatives of what I call "amic acids" and are referred to in the appended claims as "amates." The soaps referred to above are found on the market and consist of the usual compositions of long chain fatty acids with the alkali and alkaline earth metals mentioned. Thus, the fatty acids with which such metals are combined may be stearic acid, tallow fatty acids, cocoanut fatty acids, cottonseed oil fatty acids and others, or may be the soaps made by combining such metals with the whole fats per se.

The greases made in accordance with my invention may contain only small amounts of the two gelators, but nevertheless the resulting grease-like product shows an improvement over the use of modified montmorillonite grease alone, namely, it has both improved rust inhibiting properties and increased lubricity. Thus, I have employed as little as 0.5% of the combined modified montmorillonite and soap or amate gelator to give a semi-fluid grease which has the properties mentioned. Even smaller amounts of the combined gelator may be employed.

The term "lubricity" as herein employed is well understood in the art and means the ability of the lubricant to apply a lubricating film between the moving parts. Thus, the Bentone greases lack lubricity because they are unable to give up sufficient oil from the gel structure, namely, syneresis does not occur, to provide the necessary lubrication and under continued use, they will tend to channel completely without release of oil.

I have found in accordance with my invention that greases formed with petroleum lubricants as herein described may be used in varying proportions, but if it is desired to maintain the unique non-melting characteristics of the

modified montmorillonite grease, it is important that certain proportions of the various soaps and amates be employed with such montmorillonite in order to retain this non-melting characteristic.

5 These proportions are indicated in the examples given below.

The following examples represent embodiments of the invention as I now prefer to practice it. It is to be understood that the examples are illustrative and that the invention is not to be considered as restricted thereto except as indicated in the appended claims.

*Example 1.—(Mixtures using barium soap)*

15 Percent

Total gelator (composed of 81% barium stearate and 19% Bentone 34)----- 20  
300 sec./100° F. S. U. V. (Saybolt Universal viscosity) Pale Oil----- 80

20 The grease was made by making up the Bentone 34 grease and the barium stearate grease, followed by simple thorough blending of the greases at room temperature. The Bentone grease was made up by slurring 20% of Bentone 34 with one half the required oil at room temperature, sheared through a mill set at 0.001 to 0.002 inch clearance. The resultant putty-like mass was cut back with the balance of the mineral oil. The 20% barium stearate grease was made up in the usual manner.

25 These two greases were made up with the same oil, namely, the Pale Oil mentioned above. Since these greases had equivalent amounts of gelator, they were blended off in the cold in the following proportions: 81% barium stearate grease and 19% Bentone grease at room temperature.

30 The resultant Bentone-barium soap grease had the following physical properties:

35 40 D/P (dropping point) ASTM-D566 (American Society for Testing Materials)---° F--- 456  
Micro-penetration (Texas Method) at 77° F--- 99.5

The Texas Method for determining micro-penetration is well known to those skilled in the art.

45 Bentone 34 as employed in the above example is a modified montmorillonite produced as stated above and having as cations the secondary amine radicals (C<sub>18</sub>H<sub>37</sub>)<sub>2</sub>N and (C<sub>16</sub>H<sub>33</sub>)<sub>2</sub>N formed by reacting hydrated montmorillonite with technical distearyl amine.

50 It will be noted that the dropping point is stated to be 456° F. In order to determine the proportions at which no dropping point occurs, tests were made using exactly the same procedure but varying the relative proportions of the barium stearate and Bentone 34 with the following results for such dropping points and also for micro-penetration:

| Test No. | Combined Gelator        |                    | D/P, ASTM D566       | Micro-Penetration at 77° F. |
|----------|-------------------------|--------------------|----------------------|-----------------------------|
|          | Percent Barium Stearate | Percent Bentone 34 |                      |                             |
| 1-----   | 73                      | 27                 | Non-melting--do----- | 100                         |
| 2-----   | 61                      | 39                 | -----                | 90                          |

70 It will be seen from the above tests that somewhere between the ratios of barium stearate to Bentone 34 of 81% to 19% and 73% to 27%, respectively, there occurs a transition point where in the blended greases change from a grease

with melting characteristic to a grease having the non-melting characteristic.

Tests showed in each instance that the oil portion of the greases would catch fire before the grease would actually melt.

*Example 2.—(Mixtures using strontium soap)*

The following greases were made with a total combined gelator of 20% using 80% of 300 sec./-100° F. S. U. V. Pale Oil, with the following results:

| Test No. | Combined Gelator           |                    | D/P, ASTM D566 | Micro-Penetration at 77° C. |
|----------|----------------------------|--------------------|----------------|-----------------------------|
|          | Percent Strontium Stearate | Percent Bentone 34 |                |                             |
| 1        | 81                         | 19                 | 461° F.        | 63                          |
| 2        | 73                         | 27                 | Non-melting    | 94                          |
| 3        | 61                         | 39                 | do             | 99                          |

In making up the above greases, the same procedure was employed as in Example 1.

From the above data, it is to be noted that there is a ratio of strontium stearate to Bentone 34 which will give the transition point from melting to non-melting grease as described in Example 1.

*Example 3.—(Mixtures using sodium soap)*

The following greases were made with a total combined gelator of 20% using 80% of 75 sec./-210° F. S. U. V. Mid-Continent Bright Stock, with the following results:

| Test No. | Combined Gelator           |                    | D/P, ASTM D566 | Micro-Penetration at 77° F. |
|----------|----------------------------|--------------------|----------------|-----------------------------|
|          | Percent Sodium Tallow Soap | Percent Bentone 34 |                |                             |
| 1        | 75                         | 25                 | 404° F.        | 92                          |
| 2        | 67                         | 33                 | Non-melting    | 100                         |
| 3        | 57                         | 43                 | do             | 102                         |

The following greases were made with the same proportion of gelator but 80% of 100 sec./-210° F. S. U. V. Mid-Continent Bright Stock, with the following results:

| Test No. | Combined Gelator           |                    | D/P, ASTM D566 | Micro-Penetration at 77° F. |
|----------|----------------------------|--------------------|----------------|-----------------------------|
|          | Percent Sodium Tallow Soap | Percent Bentone 34 |                |                             |
| 1        | 75                         | 25                 | 383° F.        | 82                          |
| 2        | 67                         | 33                 | 383° F.        | 88                          |
| 3        | 57                         | 43                 | Non-melting    | 83                          |
| 4        | 46                         | 54                 | do             | 90                          |

The following greases were made with a total combined gelator content of 10% employing 90% of 100 sec./210° F. S. U. V. Mid-Continent Bright Stock, with the following results:

| Test No. | Combined Gelator           |                    | D/P, ASTM D566 | Micro-Penetration at 77° F. |
|----------|----------------------------|--------------------|----------------|-----------------------------|
|          | Percent Sodium Tallow Soap | Percent Bentone 34 |                |                             |
| 1        | 75                         | 25                 | 371° F.        | 108                         |
| 2        | 67                         | 33                 | 369° F.        | 117                         |
| 3        | 57                         | 43                 | Non-melting    | 128                         |
| 4        | 46                         | 54                 | do             | 120                         |

The process for making the above greases was the same as employed in Example 1.

From the above data, it is to be noted that there is a ratio of sodium tallow soap to Bentone 34 which will give the transition point from melting to non-melting grease as described in Example 1.

*Example 4.—(Mixtures using calcium soap)*

10 The following greases were made with a total combined gelator of 10% using 90% of 4000 sec./100° F. S. U. V. Coastal Cylinder Stock, with the following results:

| Test No. | Combined Gelator         |                    | D/P, ASTM D566 | Micro-Penetration at 77° F. |
|----------|--------------------------|--------------------|----------------|-----------------------------|
|          | Percent Calcium Stearate | Percent Bentone 34 |                |                             |
| 1        | 75                       | 25                 | 227° F.        | 159                         |
| 2        | 67                       | 33                 | 246° F.        | 246                         |
| 3        | 57                       | 43                 | 415° F.        | 198                         |
| 4        | 46                       | 54                 | 431° F.        | 173                         |
| 5        | 34                       | 66                 | 495° F.        | 158                         |
| 6        | 22                       | 78                 | Non-melting    | 115                         |

The following greases were made with a total combined gelator content of 20% using 80% of 100 sec./100° F. S. U. V. Pale Oil, with the following results:

| Test No. | Combined Gelator         |                    | D/P, ASTM D566 | Micro-Penetration at 77° F. |
|----------|--------------------------|--------------------|----------------|-----------------------------|
|          | Percent Calcium Stearate | Percent Bentone 34 |                |                             |
| 1        | 75                       | 25                 | 201° F.        | 84                          |
| 2        | 67                       | 33                 | 215° F.        | 94                          |
| 3        | 57                       | 43                 | 334° F.        | 93                          |
| 4        | 46                       | 54                 | 416° F.        | 89                          |
| 5        | 34                       | 66                 | 442° F.        | 96                          |
| 6        | 22                       | 78                 | Non-melting    | 86                          |

45 In making up the above greases, the same procedure was employed as in Example 1.

From the above data, it is to be noted that there is a ratio of calcium stearate to Bentone 34 which will give the transition point from melting to non-melting grease as described in Example 1.

*Example 5.—(Mixtures using lithium soap)*

55 The following greases were made with a total combined gelator content of 10% using 90% of 300 sec./100° F. S. U. V. Pale Oil, with the following results:

| Test No. | Combined Gelator         |                    | D/P, ASTM D566 | Micro-Penetration at 77° F. |
|----------|--------------------------|--------------------|----------------|-----------------------------|
|          | Percent Lithium Stearate | Percent Bentone 34 |                |                             |
| 1        | 60                       | 40                 | 391° F.        | 89                          |
| 2        | 50                       | 50                 | 425° F.        | 87                          |
| 3        | 40                       | 60                 | Non-melting    | 84                          |

70 The process for making the above greases was the same as employed in Example 1.

From the above data, it is to be noted that there is a ratio of lithium stearate to Bentone 34 which will give the transition point from melting to non-melting grease as described in Example 1.

*Example 6.—(Mixtures using sodium amate—prepared in accordance with Formula A where X is sodium, according to Serial No. 80,328)*

The following greases were prepared with a total combined gelator content of 20% using 80% of 300 sec./100° F. S. U. V. Pale Oil, with the following results:

| Test No. | Combined Gelator           |                          | D/P, ASTM<br>D566 | Micro-Pen-<br>etration<br>at 77° F. |
|----------|----------------------------|--------------------------|-------------------|-------------------------------------|
|          | Percent<br>Sodium<br>Amate | Percent<br>Bentone<br>34 |                   |                                     |
| 1        | 60                         | 40                       | 404° F.           | 107                                 |
| 2        | 50                         | 50                       | 397° F.           | 115                                 |
| 3        | 40                         | 60                       | Non-melting       | 125                                 |

In making up the above greases, the same procedure was employed as in Example 1.

From the above data, it is to be noted that there is a ratio of sodium amate to Bentone 34 which will give the transition point from melting to non-melting grease as described in Example 1.

*Example 7.—(Mixtures using strontium amate—prepared in accordance with Formula B above where M is strontium, according to Serial No. 80,328)*

The following greases were prepared with a total combined gelator content of 20% using 80% of 150 sec./210° F. Smackover Black Oil, with the following results:

| Test No. | Combined Gelator              |                          | D/P, ASTM<br>D566 | Micro-Pen-<br>etration<br>at 77° F. |
|----------|-------------------------------|--------------------------|-------------------|-------------------------------------|
|          | Percent<br>Strontium<br>Amate | Percent<br>Bentone<br>34 |                   |                                     |
| 1        | 70                            | 30                       | 455° F.           | 117                                 |
| 2        | 60                            | 40                       | Non-melting       | 140                                 |
| 3        | 50                            | 50                       | do                | 133                                 |

The process for making the above greases was the same as employed in Example 1.

From the above data, it is to be noted that there is a ratio of strontium amate to Bentone 34 which will give the transition point from melting to non-melting grease as described in Example 1.

*Example 8.—(Mixtures using barium amate—prepared in accordance with Formula B above where M is barium, according to Serial No. 80,328)*

The following greases were prepared with a total combined gelator content of 20% using 80% of 300 sec./100° F. S. U. V. Mid-Continent Neutral Oil, with the following results:

| Test No. | Combined Gelator           |                          | D/P, ASTM<br>D566 | Micro-<br>Penetration<br>at 77° F. |
|----------|----------------------------|--------------------------|-------------------|------------------------------------|
|          | Percent<br>Barium<br>Amate | Percent<br>Bentone<br>34 |                   |                                    |
| 1        | 60                         | 40                       | 392° F.           | 110                                |
| 2        | 50                         | 50                       | 395° F.           | 124                                |
| 3        | 40                         | 60                       | Non-melting       | 149                                |

The process for making the above greases was the same as employed in Example 1.

From the above data, it is to be noted that there is a ratio of barium amate to Bentone 34 which will give the transition point from melting to non-melting grease as described in Example 1.

*Example 9.—(Mixtures using lithium amate—prepared in accordance with Formula A above where X is lithium, according to Serial No. 80,328)*

The following greases were prepared with a total combined gelator of 15% using 85% of 150 sec./210° F. S. U. V. Solvent Extracted Bright Stock, with the following results:

| Test No. | Combined Gelator            |                          | D/P, ASTM<br>D566 | Micro-<br>Penetration<br>at 77° F. |
|----------|-----------------------------|--------------------------|-------------------|------------------------------------|
|          | Percent<br>Lithium<br>Amate | Percent<br>Bentone<br>34 |                   |                                    |
| 1        | 75                          | 25                       | 404° F.           | 106                                |
| 2        | 67                          | 33                       | 408° F.           | 108                                |
| 3        | 57                          | 43                       | 415° F.           | 122                                |
| 4        | 46                          | 54                       | Non-melting       | 125                                |
| 5        | 33                          | 67                       | do                | 123                                |
| 6        | 18                          | 82                       | do                | 106                                |

The process for making the above greases was the same as employed in Example 1.

From the above data, it is to be noted that there is a ratio of lithium amate to Bentone 34 which will give the transition point from melting to non-melting grease as described in Example 1.

It will be seen from the micro-penetration tests of the above examples that there are limitations on the ratio of soap or amate and Bentone which will give a minimum of weakening of Bentone gel structure. It is also evident that in some cases the effect is caused by the action of soap or amate on the Bentone. In the other cases, the Bentone affects the soap or amate gel structure. Also from the above data it can be seen that the amates affect the consistency and change to a greater extent than do the soaps.

35 30 35 40 45 The effect, however, on the consistency and gel structure of Bentone by amates is more than offset by the improvement in lubricity of the Bentone greases. This is described below under "lubricity." It is evident that the Bentone gel structure is loosened to permit more syneresis when the amates are used than when the soaps are used.

45 50 55 In ordinary practice, the gelator content of greases on the market ranges from about 5% to 25%. In special instances, the gelator content may exceed or be less than this range. In order to demonstrate the effect of increasing and decreasing the gelator content, the following tests have been made.

#### FLUID-TYPE GREASE (LOW TOTAL GELATOR CONTENT)

*Example 10.—(Mixtures using sodium soap)*

The following greases were prepared with a total combined gelator content of 1% using 99% of 150 sec./210° F. S. U. V. regular Solvent Extracted Bright Stock, with the following results:

| Test No. | Combined Gelator                    |                          | Consistency<br>at 77° F.<br>(Gardner #<br>Disc—No<br>Added<br>Weight),<br>Secs. |
|----------|-------------------------------------|--------------------------|---------------------------------------------------------------------------------|
|          | Percent<br>Sodium<br>Tallow<br>Soap | Percent<br>Bentone<br>34 |                                                                                 |
| 1        | 100                                 | 0                        | 80                                                                              |
| 2        | 75                                  | 25                       | 75                                                                              |
| 3        | 50                                  | 50                       | 70                                                                              |
| 4        | 25                                  | 75                       | 71                                                                              |
| 5        | 0                                   | 100                      | 64                                                                              |

The following greases were made up using the same ingredients as above, but with a total combined gelator content of 0.5% and 99.5% of 150 sec./216° F. S. U. V. regular Solvent Extracted Bright Stock, with the following results:

| Test No. | Combined Gelator                    |                            | Consistency at 77° F.<br>(Gardner #2 Disc—No<br>Added Weight),<br>Secs. |
|----------|-------------------------------------|----------------------------|-------------------------------------------------------------------------|
|          | Percent<br>Sodium<br>Tallow<br>Soap | Percent<br>Bentonite<br>34 |                                                                         |
| 1.....   | 100                                 | 0                          | 65                                                                      |
| 2.....   | 75                                  | 25                         | 64                                                                      |
| 3.....   | 50                                  | 50                         | 59                                                                      |
| 4.....   | 25                                  | 75                         | 60                                                                      |
| 5.....   | 0                                   | 100                        | 59                                                                      |

Examples 10 and 11 being fluid, or semi-fluid, do not have ASTM dropping points per se. The effect of the amates or soaps on the gel strength of the Bentones at elevated temperatures were determined by checking Gardner Mobilometer consistencies at temperatures above 77° F., with the following results:

| Test No. | 1% GELATOR                 |                                                  |            |
|----------|----------------------------|--------------------------------------------------|------------|
|          | Grease                     | Consistency (Gardner #2 Disc—No<br>Added Weight) |            |
|          |                            | at 100° F.                                       | at 130° F. |
| 15.....  | Example 10—Test No. 1..... | 72½                                              | 63½        |
| .....    | Example 10—Test No. 2..... | 68                                               | 58         |
| .....    | Example 10—Test No. 3..... | 64                                               | 55         |
| .....    | Example 10—Test No. 4..... | 60½                                              | 51         |
| .....    | Example 10—Test No. 5..... | 56½                                              | 47½        |
| .....    | .....                      | .....                                            | 35         |

| Test No.                   | 0.5% GELATOR |                                                  |            |
|----------------------------|--------------|--------------------------------------------------|------------|
|                            | Grease       | Consistency (Gardner #2 Disc—No<br>Added Weight) |            |
|                            |              | at 100° F.                                       | at 130° F. |
| Example 10—Test No. 1..... | 57½          | 49                                               | 33         |
| Example 10—Test No. 2..... | 55½          | 48                                               | 31         |
| Example 10—Test No. 3..... | 54           | 45                                               | 32         |
| Example 10—Test No. 4..... | 52           | 42½                                              | 31½        |
| Example 10—Test No. 5..... | 51½          | 42½                                              | 30         |

| Test No.                   | 1% GELATOR |                                                  |            |
|----------------------------|------------|--------------------------------------------------|------------|
|                            | Grease     | Consistency (Gardner #2 Disc—No<br>Added Weight) |            |
|                            |            | at 100° F.                                       | at 130° F. |
| Example 11—Test No. 1..... | 58         | 49                                               | 33         |
| Example 11—Test No. 2..... | 56½        | 46                                               | 32½        |
| Example 11—Test No. 3..... | 55½        | 45½                                              | 31½        |
| Example 11—Test No. 4..... | 53½        | 45½                                              | 32         |
| Example 11—Test No. 5..... | 54         | 45                                               | 32         |
| Example 11—Test No. 6..... | 51         | 42                                               | 30         |

| Test No.                   | 0.5% GELATOR |                                                  |            |
|----------------------------|--------------|--------------------------------------------------|------------|
|                            | Grease       | Consistency (Gardner #2 Disc—No<br>Added Weight) |            |
|                            |              | at 100° F.                                       | at 130° F. |
| Example 11—Test No. 1..... | 47½          | 39                                               | 26½        |
| Example 11—Test No. 2..... | 48½          | 39                                               | 26         |
| Example 11—Test No. 3..... | 47½          | 38½                                              | 25½        |
| Example 11—Test No. 4..... | 47½          | 38                                               | 25         |
| Example 11—Test No. 5..... | 47½          | 38½                                              | 26½        |
| Example 11—Test No. 6..... | 47           | 37½                                              | 25         |

When the above data are graphed using rectangular coordinates, it can be seen that the values fall within the limits required for linearity. Therefore the gel strength is unimpaired at elevated temperatures as well as at room temperature.

50 HIGH GELATOR CONTENT GREASE

Example 12.—(Mixtures using sodium amate—Prepared as in Example 6)

The following greases were prepared with a total combined gelator content of 35% using 65% of 300 sec./100° F. S. U. V. Pale Oil, with the following results:

| Test No. | Combined Gelator            |                            | Consistency at 77° F.<br>(Gardner #2 Disc—No<br>Added Weight), secs. |
|----------|-----------------------------|----------------------------|----------------------------------------------------------------------|
|          | Percent<br>Lithium<br>Amate | Percent<br>Bentonite<br>34 |                                                                      |
| 1.....   | 100                         | 0                          | 54                                                                   |
| 2.....   | 70                          | 30                         | 54                                                                   |
| 3.....   | 55                          | 45                         | 59                                                                   |
| 4.....   | 45                          | 55                         | 59                                                                   |
| 5.....   | 30                          | 70                         | 52                                                                   |
| 6.....   | 0                           | 100                        | 54                                                                   |

  

| Test No. | Combined Gelator           |                            | D/P, ASTM<br>D566 | Micro-<br>Penetration<br>at 77° F. |
|----------|----------------------------|----------------------------|-------------------|------------------------------------|
|          | Percent<br>Sodium<br>Amate | Percent<br>Bentonite<br>34 |                   |                                    |
| 60.....  | 70                         | 30                         | Non-melting       | 36                                 |
| 65.....  | 50                         | 50                         | do                | 31                                 |

The process for making the above greases was the same as employed in Example 1.

Example 13.—(Mixtures using lithium amate—Prepared as in Example 9)

The following greases were prepared with a total combined gelator content of 35% using 65%

It can be seen that at 77° F. for the 0.5% gelator concentration there is no diminution of gel strength, the same being true for the 1% concentration.

The process for making the above greases was the same as employed in Example 1.

of 150 sec./210° F. S. U. V. Solvent Extracted Bright Stock, with the following results:

| Test No. | Combined Gelator      |                    | D/P, ASTM D566 | Micro-Penetration at 77° F. |
|----------|-----------------------|--------------------|----------------|-----------------------------|
|          | Percent Lithium Amate | Percent Bentone 34 |                |                             |
| 1-----   | 70                    | 30                 | Non-melting    | 35                          |
| 2-----   | 50                    | 50                 | do             | 32                          |

Examination of the data reported for Examples 12 and 13 indicates that high total gelator content greases are even more stable than greases made with lower total gelator content.

It has been found in accordance with the tests given below that the mixtures of soaps or amates with Bentone 34 improved the inhibition to rusting, as well as the lubricity as compared with the ordinary Bentone greases. The following rusting tests using the Army-Navy Grease Specification No. 25A described Humidity Cabinet, run at 100° F. ± 2° F. at 100 relative humidity, using the lowest concentration of soap or amate reported in the above examples, were made:

| Grease                                                                                                                  | Hours to Failure |
|-------------------------------------------------------------------------------------------------------------------------|------------------|
| Blank (bare metal untreated).....                                                                                       |                  |
| 10% Bentone Grease with 300 sec./100° F. S. U. V. Pale Oil.....                                                         | 4                |
| Example 1.....                                                                                                          | 23/4             |
| Example 2—Test No. 3.....                                                                                               | 300              |
| Example 3—Test No. 3 (20% total combined gelator with 75 sec./210° F. S. U. V. Mid-Continent Bright Stock).....         | 312              |
| Example 3—Test No. 4 (20% total combined gelator with 100 sec./210° F. S. U. V. Mid-Continent Bright Stock).....        | 401              |
| Example 3—Test No. 4 (10% combined total gelator with 90% of 100 sec./210° F. S. U. V. Mid-Continent Bright Stock)..... | 297              |
| Example 4—Test No. 6 (10% combined total gelator with 90% 4,000 sec./100° F. S. U. V. Coastal Cylinder Stock).....      | 305              |
| Example 4—Test No. 6 (20% combined total gelator with 80% 100 sec./100° F. S. U. V. Pale Oil).....                      | 79               |
| Example 5—Test No. 3.....                                                                                               | 40               |
| Example 6—Test No. 3.....                                                                                               | 62               |
| Example 7—Test No. 3.....                                                                                               | 590              |
| Example 8—Test No. 3.....                                                                                               | 615              |
| Example 9—Test No. 6.....                                                                                               | 410              |
| Example 10—Test.....                                                                                                    | 465              |
| 2 Controls for Example 10 10% of Bentone grease with 300 sec./100° F. S. U. V. Pale Oil.....                            | 521              |
| Example 11—Test.....                                                                                                    | 21               |
| 2 Controls for Example 11 10% of Bentone grease with 300 sec./100° F. S. U. V. Pale Oil.....                            | 2                |
| Example 12—Test 2.....                                                                                                  | 48               |
| Example 13—Test 2.....                                                                                                  | 2                |
| 1 Control for Examples 12 and 13 10% of Bentone grease with 300 sec./100° F. S. U. V. Pale Oil.....                     | over 700         |
|                                                                                                                         | over 700         |
|                                                                                                                         | 4                |

Examples 10 and 11 show marked improvement in rust resistance as compared with Bentone alone even though these examples have a very low content of gelator. The increase in total gelator to 35% shown in tests of Examples 12 and 13 produces a great increase in rust inhibition.

The lubricity improvement was demonstrated by using the Falex machine made by Faville-Levalley Corporation of Chicago, Illinois. The straight Bentone grease would only carry 200 lbs. gauge, whereas the soap diluted greases carried 350 lbs., and the amates 450 lbs. gauge, in all cases.

From the above data as given in the examples and tests, it will be noted that the objectionable properties of the Bentone greases, namely, their tendency to rust, may be overcome by combining these greases with one or more of the following: barium, strontium, sodium, calcium and lithium soap greases and barium, strontium, sodium and lithium "amates." I have found that these mix-

tures while preserving all of the beneficial characteristics such as high dropping point of the Bentone grease, also add the beneficial characteristics of high resistance to rusting and greatly improved lubricity.

What I claim is:

1. A lubricating composition of a petroleum lubricant, a montmorillonite modified by an organic cation, and a long-chain organic salt gelator which contains a straight chain of at least 8 carbon atoms and whose salt-forming metal is selected from the group consisting of lithium, sodium, calcium, barium, and strontium, said organic salt having the characteristic of improving the lubricity and inhibiting the rust-producing properties of the modified montmorillonite, the proportions of modified montmorillonite to said organic salt gelator ranging from 19-78% of said modified montmorillonite to 81-22% of said organic salt gelator.
2. A composition in accordance with claim 1 in which the combined modified montmorillonite and organic salt gelator are present in the proportion of at least 0.5%.
3. A grease compound of a petroleum lubricant and a gelator comprising not more than about 81% to 73% barium soap and not less than about 19% to 27% modified montmorillonite.
4. A grease compound of a petroleum lubricant and a gelator comprising not more than about 75% to 57% sodium soap and not less than about 25% to 43% modified montmorillonite.
5. A grease compound of a petroleum lubricant and a gelator comprising not more than about 60% to 40% lithium soap and not less than about 40% to 60% modified montmorillonite.
6. A grease compound of a petroleum lubricant and a gelator comprising not over about 60% to 40% sodium "amate" and not less than about 40% to 60% modified montmorillonite.
7. A grease compound of a petroleum lubricant and a gelator comprising not over about 75% to 46% lithium "amate" and not less than about 25% to 54% modified montmorillonite.
8. A grease compound of a petroleum lubricant and a gelator comprising not more than about 81% to 73% barium stearate and not less than about 19% to 27% modified montmorillonite.
9. A grease compound of a petroleum lubricant and a gelator comprising not more than about 75% to 57% neutral sodium tallow soap and not less than about 25% to 43% modified montmorillonite.
10. A grease compound of a petroleum lubricant and a gelator comprising not more than about 60% to 40% lithium stearate and not less than about 40% to 60% modified montmorillonite.
11. A grease compound of a petroleum lubricant and a gelator comprising not over about 60% to 40% sodium N-lauryl sebacamate and not less than about 40% to 60% modified montmorillonite.
12. A grease compound of a petroleum lubricant and a gelator of not over about 75% to 46% lithium N-lauryl sebacamate, and not less than 25% to 54% modified montmorillonite.

WILLIAM C. BRYANT.

References Cited in the file of this patent  
UNITED STATES PATENTS

Number Name Date  
75 2,531,440 Jordan Nov. 28, 1950